

W. M. PAGE.  
REINFORCED COPPER AND PROCESS OF MAKING THE SAME.  
APPLICATION FILED JUNE 28, 1911.

1,125,163.

Patented Jan. 19, 1915.



Inventor

*W. M. Page*

Witnesses

*H. C. Robielle*  
*R. F. Steeward*

By

*K. P. McElroy*

Attorney

# UNITED STATES PATENT OFFICE.

WILLIAM MARSHALL PAGE, OF RIDLEY PARK, PENNSYLVANIA.

## REINFORCED COPPER AND PROCESS OF MAKING THE SAME.

1,125,163.

### Specification of Letters Patent.

Patented Jan. 19, 1915.

Application filed June 23, 1911. Serial No. 634,887

*To all whom it may concern:*

Be it known that I, WILLIAM MARSHALL PAGE, a citizen of the United States, residing at Ridley Park, in the county of Delaware and State of Pennsylvania, have invented certain new and useful Improvements in Reinforced Copper and Processes of Making the Same, of which the following is a specification.

10 This invention relates to reinforced copper and processes of making the same; and it comprises a body of reinforced copper, such as a conductor wire, having distributed through it a plurality of spaced and isolated linear reinforcing bodies of relatively small diameter and in substantially parallel alignment, such reinforcing bodies consisting of a strong cupriferous alloy, being weld-united to the copper of the main body  
15 and having the characteristics of pre-worked metal; and it also comprises a process of producing such reinforced copper wherein a strong cupriferous alloy, such as vanadium bronze, aluminum bronze, silicon  
20 bronze, phosphorus bronze, etc., is converted into rods or the like, a plurality of such rods are spaced apart in a substantially parallel arrangement in a suitable mold and at a distance from the walls of such mold,  
25 copper is cast around and among such rods to unite therewith and form a compound billet, and the billet is worked down to rod or wire; and it also comprises a process wherein rods or the like made from such  
30 copper are cast around and among them to unite therewith and form a compound billet, and the billet is worked down to rod or wire; and it also comprises a process wherein rods or the like made from such  
35 copper are in turn used as reinforcing bodies or elements in making a secondary billet, such primary rods being placed in a mold as before, copper cast around and among them to unite therewith  
40 and form a secondary billet and this secondary billet in turn worked down to rod or wire; the secondary rod so produced being, if desired, in turn used to produce a tertiary billet, and so on; all as more  
45 fully hereinafter set forth and as claimed.

Pure copper is the most desirable commercially available metal for electric conductors because of its high conductivity but it is a weak metal with a low elastic limit. When it is strengthened by alloying with tin and other metals, it loses greatly in conductivity. With its low elastic limit, when copper is used for hung and strung wires it is apt to sag and neck under temperature changes; copper once stretched beyond the elastic limit not regaining its orig-

inal section. Hard drawing copper wire gives it more strength, but does not do away with the low elastic limit.

In the present invention it is an object 50 to produce a compound body of metal which shall unite a high conductivity approximating that of copper with a comparatively high tensile strength and elastic limit. For this purpose a main body of copper is used 65 in a substantially pure state and this main body is reinforced with a plurality of distributed relatively fine linear threadlike bodies or elements of a stronger copper alloy, such as bronze. While the various 70 bronzes have a low conductivity as compared with copper, their conductivity is high as compared with that of other strong metals, such as steel. Therefore a relatively large amount of bronze reinforcement can 75 be used without running down the conductivity unduly. Each reinforcing element should however be relatively minute in cross section, the desired amount of reinforcement being best obtained by multiplying the number of reinforcements rather than by increasing their relative size. By using the 80 alloy as a multiplicity of threadlike bodies, not only is more strength attained but undue stiffness is avoided. By using a strong 85 reinforcing alloy in the form of a multiplicity of relatively fine linear threads the flexibility of the copper is not much interfered with. A compound or reinforced copper wire can be produced which, while relatively flexible and easily handled and not 90 springy, is nevertheless possessed of great tensile strength. A much higher conductivity in a copper wire can be secured by using a small amount of tin or other 95 strengthening metal in distributed bodies of alloy in threadlike reinforcing arrangement than by incorporating the same amount of tin with the whole body of the wire. In the present invention I secure a 100 compound wire or the like having longitudinal veins, layers, laminae or strata of pure copper with other layers, veins or the like of copper strengthened by alloying. The alloy, instead of permeating the whole 105 mass of material, thus occurs in restricted included strengthening ribs or linear bodies; linear bodies which have the properties of worked metal.

In working the stronger copper alloys such as vanadium bronze, silicon bronze, phosphorus bronze, aluminum bronze, etc.,

to rod and wire, each successive working gives an increase in tensile strength and other desirable properties; an increase which is not wholly done away with by subsequent heat treatment, annealing and the like. The good effect of working remains with the metal until it is finally melted up. Therefore by converting the stronger copper alloys into relatively strong worked-down rods and using a plurality of these rods as cores in making an ingot of copper, the alloys are used in a mechanically strong form, while the further reduction to rod and wire of the new ingot or billet so formed still further improves the strength and mechanical qualities of the included linear reinforcements. The rods, in any number and arrangement desired, may be placed in a mold and copper cast around and among them in such a manner as to weld therewith to form a compound ingot or billet. This ingot may then be drawn down. In working down, as stated, the included strong copper rods are further reduced to wire-like or threadlike fineness and in this reduction, their tensile strength and other valuable properties are very much improved. Presuming, for example, that a strong phosphor bronze or vanadium bronze is cast into a billet of, say, 6 or 8 inches diameter, and this worked down by rolling to, say, 0.291 inch in diameter rod, the strength of the bronze will be very much heightened and the physical qualities improved in this working. Assuming, now, that this rod is placed in a mold of, say, 6 $\frac{1}{2}$  inches in diameter and copper cast around it in such a manner as to weld unite with it, and then the compound billet in turn is drawn down to another rod of 0.291 inch, it will be obvious that the original billet of phosphor bronze has been reduced to threadlike fineness; it has been worked down very far and its mechanical properties concomitantly improved. It will be in fact about 0.0002 inch in diameter. And if this rod be now drawn to a fine wire, the thickness of the included bronze thread is once more reduced and its strength improved. What is true of a single core rod in this example is true of each of the 50 or 100 rods which may be used as included cores in making a composite billet under the present invention. Each of these rods will be worked to a linear wire-like or threadlike body of very strong metal. In the new rod or wire worked down from the compound billet each original rod will have been converted into a threadlike reinforcing body and while the thickness of each of these linear bodies is infinitesimal, there will ordinarily be a great many of them so as to give a total sectional area of as many per cent. as desired; enough, say, to give the new rod or wire 10, 15, or 20 per cent. of aluminum bronze, vanadium

bronze, silicon bronze or phosphor bronze. Supposing the amount be 20 per cent., then one-fifth of the mass will be bronze but this one-fifth part of the mass will not occur as a single comparatively rigid core, but as a multiplicity of relatively flexible, relatively strong filaments. Where the amount of the reinforcing metal is heightened considerably to say, 50 to 60 per cent. of the total amount, a new and interesting material is formed; a material which combines high tensile strength and high elastic limit with a comparative lateral flexibility. The nearest material with which it can be compared is possibly a stranded cable. As is well known, a bar of any metal of a given cross section, say, an inch, is not as strong as the same metal converted into fine wires and these wires stranded together to make a rope of the same given cross section, say, again, an inch. This is true of bronze, of steel, and of most other metals. Now in the present material, the bronze has been reduced, in most cases, to filaments very much finer than can be produced by ordinary wire drawing processes and with a concomitant heightening in strength. For a given unit of cross section, any of these filaments is much stronger than the metal of an ordinary wire of the same material. A multiplicity of these filaments in the new material instead of being stranded together mechanically, as in a wire rope, are set side by side in a substantially parallel alinement and are spaced and united by soft copper. The properties of such a composite metal are unique in the arts. For the purposes of electrical conductors it is not desirable to have a high production of reinforcing metal; to have a greater proportion of reinforcing filaments than is necessary to secure the combination of conductivity, from the copper, and of strength, from the bronze threads. As stated however the bronzes are relatively good conductors. In making a compound billet or ingot, any suitable type of mold may be employed. There are some advantages in providing it with means for maintaining it full of an indifferent gas, such as nitrogen or producer gas. Steam may also be used since it is almost indifferent to copper and cupriferous alloys. The reinforcing rods may be of any number or shape or section desired. They may be rounds, squares, ovals, octagons, hexagons, etc. Whatever their shape, the same shape will substantially reappear in the filaments of the drawn down material. Where stiffness is desired with a minimum amount of reinforcing metal, the original rods employed may be channels or of I or T section. However, round rods are suitable for most purposes. Reinforcements of stranded rope or cable may be used, and particularly where it is desired to obtain very

fine threads in the resultant material with a small amount of reduction. But this is not ordinarily advisable since stranded wire is more expensive than plain rods; and it is 5 furthermore difficult to cast low-temperature copper around a stranded metal reinforcement without leaving air-filled cavities which in the resultant material will elongate into linear flaws. Prior to placing in the 10 mold, the surface of the rod may be sand-blasted or pickled to give it a true metallic surface. This promotes union with the copper subsequently cast in. Occasionally, for 15 certain electrical purposes, it is desirable to have the rods not weld united with the main body of the copper, but discrete therefrom; and for purposes such as this, the surfaces of the rods may be oxidized somewhat. But ordinarily it is better to have the rods 20 bright-surfaced and produce a weld union. The copper cast around and among the rods in the mold, for electrical purposes, should be as pure as possible; and it should be cast in at a relatively low temperature so as to 25 avoid melting down the bronze or destroying the integrity of the rods. Water-cooled iron molds may be used or the mold may have thick walls of conductive material. A useful type of mold is made by casting a 30 heavy copper ring around a steel or iron mold. In forming a compound ingot the copper cast in ordinarily should be as pure as possible and with heat conductive molds and with rods spaced away from its walls, 35 a ring of pure copper may be first solidified next such walls while molten copper still occurs at the center among the rods. The rods may be clustered or placed in the mold in any arrangement desired. For some 40 purposes it is convenient to have a single series of rods in annular arrangement; but for others they may be clustered centrally. Arrangement in stars and other geometrical forms is not usually worth while. But 45 however they are spaced and placed in the mold, there should always be a free space around the assemblage of rods to allow the formation of a shell of pure copper; that is, all the rods should be placed at points re- 50 moved from the inner periphery of the mold. The number and size of rods may be as desired. The smaller the rods, the finer will be the reinforcing filaments in the ultimate rods or wire with a given amount of 55 reduction. For many purposes, the use of one-half inch or three-eighths inch rods in making ordinary size round billets, say, 6 to 7 inch billets, is convenient. Where a still greater reduction of the bronze rein- 60 forcements is required, it is often convenient and advantageous to make a primary billet in the way just described, reduce it to rods, say, three-eighth inch rods, and use these reinforced primary rods as reinforce- 65 ments for a new, or secondary, billet. Such

reinforced rods may be spaced in a mold as before, copper once more cast about and among them to form a new or secondary billet and this secondary billet in turn drawn down to rod or wire. The process may of course be repeated to form tertiary, quaternary, etc., billets, rods and wire. 70

Any of the commercial stronger bronzes may be employed for the present purposes. The brasses may also be used but do not 75 draw and work as well as the bronzes. A good bronze for the present purposes has 1.5 to 4 per cent. tin with 98.95 per cent. of copper, the residual .05 per cent. consisting of silicon, manganese, phosphorus, etc., according to the type of bronze used. Vanadium bronzes, which are extremely strong, are well suited for my purposes. A small amount of vanadium will greatly toughen 80 copper. Aluminum bronze is also very 85 suitable.

Supposing a 0.291 inch bronze rod used in making a 6 $\frac{1}{2}$  primary billet, and this billet in turn reduced to 0.291 rod the original rod in the new wire will be reduced to a diameter of about .0002, which is extremely fine. If the primary rod be employed in 90 making a new or secondary compound 6 $\frac{1}{2}$  inch billet and this in turn drawn to 0.291 rod, the original bronze rod will now be reduced to a diameter of approximately .00000066 inch. With bronze threads so 95 extremely fine as these in either the primary wire or in the secondary wire, and with a multiplicity of such fine threads clustered 100 together in parallel arrangement, it will be obvious that a new and interesting type of material is produced.

In the accompanying illustration I have 105 shown, more or less diagrammatically, certain means and material in the present invention.

In this showing Figure 1 is a vertical section of a simple type of mold containing copper and reinforcing bodies; Fig. 2 is a section of a billet containing annularly arranged reinforcements; Fig. 3 is a similar view of a wire drawn from the material of Fig. 5; Fig. 4 is a similar view of a billet containing reinforcements clustered in several annular rows; Fig. 5 is a similar view of a billet having the reinforcements clustered at the center; Fig. 6 is a similar view of a billet with the reinforcements in star arrangement; Fig. 7 is a section of a reinforced secondary billet containing reinforcements derived from a primary billet. Fig. 8 is a horizontal section of a flat sheet bar having crossed reinforcements, and Fig. 9 is a vertical transverse section of the same on line x-x. 110 115 120 125

In the showing of Fig. 1 element 1 is a simple type of mold on base plate 2 and having top 3. Through this top passes a pouring hopper 4. Inlet 5 may serve for the in- 130

5  
troduction of indifferent gas, and outlet 6  
for the exit of gas. The mold is shown as  
containing a body 7 of cast copper and rods  
8 of worked cupriferous alloy, such as van-  
adium bronze, aluminum bronze, etc.

10  
In the showing of Figs. 2, 3, 4, 5 and 6,  
the integral copper body is designated as be-  
fore by 7, while 8 represents the reinforce-  
ments.

15  
In Fig. 7, the integral copper body is  
shown as containing reinforcing elements 9,  
each of which in turn contains reinforce-  
ments 10.

20  
While my invention is particularly useful  
in making rods, wires and the like, and par-  
ticularly for conductor purposes, it is also  
applicable for the manufacture of sheets,  
tubes and other shapes. For many purposes  
25  
for which copper is used in the arts, because  
of its non-corrodibility, such as evaporating  
devices and the like, it is desirable to have it  
of somewhat stronger character. The size  
of a vacuum pan, for example, is limited by  
the structural strength of copper in avail-  
25  
able sizes. A vacuum pan must withstand  
atmospheric pressure and if the pan be over  
a given size, copper sheets cannot be relied  
upon to furnish the strength unless of undue  
thickness and weight. Metal sheets for such  
30  
purposes must be like copper, capable of be-  
ing worked into shape under the hammer;  
the metal must be malleable and flow under  
the tool. By reinforcing copper with bronze  
in the present invention sheets can be ob-  
35  
tained which combine a high tensile strength  
with a flowability like that of copper. For  
this purpose instead of using only longitudi-  
nal reinforcing elements it is better to have  
reinforcing elements in two directions.  
40  
That is, instead of merely clustering longi-  
tudinal rods in a mold and casting copper  
about them, it is better to use rods arranged  
in two directions. The rods may, and very  
usefully for many purposes, be interlaced in  
45  
a sort of open fabric. Presuming that  
strengthening rods of material, such as de-  
scribed, be woven into a sort of loose or open  
fabric, that is in right-angled arrangement,  
copper cast about them to form a compound  
50  
billet and then rolled down into sheets, an  
article will be secured which is substantially  
copper so far as its hammering properties  
are concerned, but nevertheless has a greater  
degree of strength than copper alone can  
55  
have. If the reinforcements be, as is prefer-  
able, each of relatively small diameter as re-  
gards the body of copper, on cutting the  
new reinforced sheet to sizes such as are de-  
sired, there will be merely spots of alloy ex-  
60  
posed.

65  
Reinforced bars or sheets such as de-  
scribed, which may have reinforcements dis-  
tributed through the bar or sheet in one or  
more planes, may of course be converted into  
structural elements, such as T's, I's, chan-

nels, cross-sectioned elements, etc. For such  
material of course perforated plates of  
strong metal, "expanded metal," or electric-  
ally welded woven screen as well as ordi-  
nary woven screen material may be em-  
ployed. But the product, using such mate-  
rials, does not have the reinforcements  
spaced and isolated from each other at all  
points.

70  
In Figs. 8 and 9 I have shown a sheet bar  
adapted for the described purpose. In this  
showing a flat sheet bar 7 of copper has in-  
corporated therein strengthening rods 8 of  
copper alloy. As shown these strengthen-  
ing rods extend in two directions and are in-  
terwoven into a sort of loose or open fabric.

75  
Aluminum bronze is extremely suitable as  
reinforcing metal for producing a strong  
copper article with a high scrap value.  
80  
Aluminum bronze in and of itself is one of  
the strongest of the cupriferous alloys,  
working and drawing well. When used as  
the reinforcing rods under the present in-  
vention a very strong reinforced copper is  
85  
produced, with a high conductive value, and  
with a high scrap value. On re-melting  
such reinforced metal the aluminum can be  
readily burnt out, leaving a substantially  
pure copper. Or, the scrap reinforced metal  
90  
may have a little additional aluminum  
added to it, to make aluminum bronze of the  
correct proportions, be cast into billets, con-  
verted into rods, and used anew.

95  
What I claim is:—

100  
1. The process of making reinforced metals  
which comprises assembling a plurality of  
isolated rods of a strong, worked cupriferous  
alloy in substantially parallel alinement in  
a suitable mold and casting a body of copper  
105  
into said mold around and among said rods.

2. The process of making reinforced metals  
which comprises assembling a plurality of  
isolated rods of a strong worked bronze in  
substantially parallel alinement in a suitable  
mold and casting a body of copper into said  
110  
mold around and among said rods in such a  
manner as to produce a superficial union  
with said rods.

3. The process of making reinforced metals  
which comprises assembling a plurality of  
isolated rods of a strong worked cupriferous  
alloy in substantially parallel alinement in a  
suitable mold and casting cupriferous metal  
115  
into said mold around and among said rods  
in such a manner as to produce a superficial  
union with said rods.

120  
4. The process of making reinforced metals  
which comprises assembling a plurality of  
isolated rods of a strong, worked cupriferous  
alloy in substantially parallel alinement  
125  
in a suitable mold and casting copper into  
said mold around and among said rods in  
such a manner as to produce a superficial  
union with said rods and working down the  
composite billet so formed.

5. The process of making reinforced metals which comprises assembling a plurality of isolated rods of a strong worked bronze in substantially parallel alinement in a suitable mold and casting copper into said mold around and among said rods in such a manner as to produce a superficial union with said rods and working down the composite billet so formed. 60
- 10 6. The process of making reinforced metals which comprises assembling a plurality of isolated rods of a strong worked cupriferous alloy in substantially parallel alinement in a suitable mold and casting a cupriferous metal into said mold around and among said rods in such a manner as to produce a superficial union with said rods and working down the composite billet so formed. 65
- 15 7. The process of making reinforced metals which comprises assembling a plurality of isolated rods of a strong worked cupriferous alloy in substantially parallel alinement in a suitable mold and casting a cupriferous metal into said mold around and among said rods in such a manner as to produce a superficial union with said rods, working down the composite billet so formed to produce rodlike bodies, placing said rodlike bodies in a mold in spaced arrangement, and casting 70 copper into said mold to produce a secondary billet. 75
- 20 8. The process of making reinforced metals which comprises assembling a plurality of isolated rods of a strong worked cupriferous alloy in substantially parallel alinement in a suitable mold and casting copper into said mold around and among said rods, working down the composite billet so formed to produce rodlike bodies, placing said rodlike bodies in a mold in spaced arrangement, casting copper into said mold to produce a secondary billet and working down such 80 secondary billet. 85
- 25 9. A reinforced copper article comprising a body of copper and a plurality of isolated substantially parallel linear elements of strong cupriferous alloy having the properties of worked metal distributed through and weld-united to said body. 90
- 30 10. A reinforced copper article comprising a body of copper and a plurality of isolated substantially parallel linear elements of a bronze having the properties of worked metal distributed through and weld-united to said body. 95
- 35 11. A reinforced copper article comprising a body of copper and a plurality of isolated substantially parallel linear threadlike elements of a strong cupriferous alloy having the properties of worked metal, distributed through and weld-united to said body, each of said elements being of relatively minute diameter as compared with the diameter of said body of copper. 100
- 40 12. A reinforced copper article comprising a body of copper and a plurality of isolated substantially parallel linear threadlike elements of bronze having the properties of worked metal distributed through and weld-united to said body, each of said elements being of relatively minute diameter as compared with the diameter of said body of copper. 105
- 45 13. A reinforced elongated copper article comprising a shell of copper and an interior composed of a plurality of isolated substantially parallel linear bodies of alloyed copper spaced and united by pure copper, said alloyed copper having the properties of worked metal. 110
- 50 14. A reinforced copper article comprising a body of copper and a plurality of incorporated isolated substantially parallel linear reinforcing elements weld-united to the main body of copper, each of said reinforcing bodies having the properties of worked metal and comprising a plurality of linear, threadlike bodies of strong cupriferous alloy spaced and united by copper weld-united thereto. 115
- 55 15. A reinforced copper article comprising a body of copper and a plurality of incorporated isolated substantially parallel linear reinforcing elements weld-united to the main body of copper, each of said reinforcing elements having the properties of worked metal and comprising a plurality of isolated linear, threadlike bodies of bronze spaced and united by copper weld-united thereto. 120
- 60 16. An integral metal article having a body of substantially pure copper inclosing, spacing and uniting a plurality of isolated substantially parallel elongated bodies of alloyed copper. 125
- 65 In testimony whereof, I affix my signature in the presence of two subscribing witnesses. 130
- 70 WILLIAM MARSHALL PAGE.
- 75 Witnesses:  
K. P. McELROY,  
FRANK R. CHAMBERS, Jr.